

March 21, 1933.

H. SCOTT

1,902,589

BIMETAL THERMOSTAT

Filed April 23, 1930



WITNESSES:

*R.J. Fitzgerald*  
*N.M. Buebel*

INVENTOR

Howard Scott.  
BY  
*Berkeley K. Carr*  
ATTORNEY

## UNITED STATES PATENT OFFICE

HOWARD SCOTT, OF WILKINSBURG, PENNSYLVANIA, ASSIGNOR TO WESTINGHOUSE ELECTRIC & MANUFACTURING COMPANY, A CORPORATION OF PENNSYLVANIA

## BIMETAL THERMOSTAT

Application filed April 23, 1930. Serial No. 446,776.

My invention relates to thermal devices and particularly to bi-metallic thermostats.

An object of my invention is to provide a bi-metallic thermostat that shall have substantially all of the following characteristics; first, that it shall be operable up to a relatively high temperature; second, that it shall have a relatively high sensitivity or deflection over a predetermined and rather large range of temperature; third, that it shall be easily rolled or otherwise fabricated.

In practicing my invention, I provide a bi-metal thermostat including a high-expansion member containing a major portion of iron, appreciable but minor quantities of manganese and nickel, and relatively small quantities of silicon and carbon, while the low expansion member is an alloy containing a major portion of iron, minor quantities of nickel and cobalt and very small quantities of manganese and carbon.

The single figure of the drawing is a sectional view of a bi-metal bar embodying my invention.

Since the operating temperatures to which bi-metallic thermostats are being subjected are increasing, it is necessary to provide a combination of high-expansion and low-expansion members which shall not lose their strength at relatively high temperatures, and shall have a composition which will ensure that the thermostat will operate in the same manner and to the same extent even after a relatively large number of cyclic operations.

I have found that austenitic iron alloys have high expansivity and high strength at the higher temperatures, and an alloy of this kind may be obtained by alloying a major portion of iron with minor portions of manganese and nickel and lesser quantities of silicon and carbon. Carbon can be used in alloys of this kind in relatively small quantities only because, if it is used in larger quantities, it introduces non-reversible expansion

of the alloy. If manganese alone is utilized, it will result in two difficulties, namely, an irreversible transformation near ordinary temperature values and a higher hardness in the high-expansion member than is present in the low-expansion member.

In the drawing, a high-expansion member 11, of the composition hereinafter set forth is closely united with a low-expansion member 12, of the composition set forth below. The completed thermostat may, of course, take any one of a number of forms.

Herewith is a table of representative combinations of materials used in the high-expansion member and in the low expansion member, respectively, of my new bi-metal combination.

## High-expansion member

| No. | Per cent Mn | Per cent Si | Per cent C | Per cent Ni | Remainder | 65 |
|-----|-------------|-------------|------------|-------------|-----------|----|
| (1) | 12.-22.     | 0.1-0.5     | 0.1-0.3    | 1-5         | Fe+impur. |    |
| (2) | 13.5        | 0.2         | 0.2        | 5.9         | Fe+impur. |    |
| (3) | 20.0        | 0.2         | 0.2        | 3.          | Fe+impur. |    |
| (4) | 17.0        | .01         | 0.4        | 5.          | Fe+impur. |    |
| (5) | 12.0        | 0.1         | 0.2        | 8.          | Fe+impur. |    |
| (6) | 10.0        | 0.1         | 0.2        | 10.0        | Fe+impur. | 70 |

## Low-expansion member

| No. | Per cent Ni | Per cent Co | Per cent Mn | Per cent C | Remainder | 75 |
|-----|-------------|-------------|-------------|------------|-----------|----|
| (1) | 41.-45.     | <2.0        | 0.2-0.9     | 0-0.3      | Fe+impur. |    |
| (2) | 42.0        | <2.0        | 0.7         | 0.1        | Fe+impur. |    |
| (3) | 44.0        | <2.0        | 0.7         | 0.1        | Fe+impur. |    |
| (4) | 26.-30.     | 11.-19.     | 0.2-0.9     | 0.1-0.3    | Fe+impur. |    |
| (5) | 27.8        | 14.2        | 0.7         | 0.1        | Fe+impur. |    |
| (6) | 26.7        | 17.3        | 0.7         | 0.1        | Fe+impur. |    |
| (7) | 29.4        | 12.6        | 0.2         | 0.1        | Fe+impur. | 80 |
| (8) | 28.3        | 15.7        | 0.2         | 0.1        | Fe+impur. |    |

I have found that the addition of nickel to a ferrous alloy containing a minor percentage of manganese has the effect of substantially eliminating the delta to gamma transformation of the iron within the temperature range of from 0° C. to substantially 500° C., and I have found that combinations of alloys such as are set forth in the tables here- 90

inbefore given can be easily fabricated, that is, rolled, for the reason that the hardness of the two elements is substantially the same. The deflection of such bi-metal combinations is relatively high, but the major characteristic which is inherent in these alloys is that of improved work hardening properties so that it is much easier to manufacture and fabricate bi-metals of this kind than has been possible heretofore.

10 Various modifications may be made in the device embodying my invention and I desire, therefore, that it shall be limited only by the appended claims.

15 I claim as my invention:

1. A thermostatic element comprising a pair of cooperating metallic members having different temperature coefficients of expansion, the high-expansion member including 20 approximately sixteen per cent of manganese, a major portion of iron, relatively small quantities of silicon and carbon and approximately three per cent of nickel to substantially eliminate the delta to gamma transformation 25 of the iron within the temperature range of from 0° C. to 500° C., and the low-expansion member being an iron alloy including approximately twenty-eight per cent nickel, approximately sixteen per cent cobalt and 30 not over one per cent each of manganese and carbon.

2. A thermostatic element including a pair of cooperating metallic members having different temperature coefficients of expansion, 35 the high-expansion member having substantially the following composition,

|           | Per cent  |
|-----------|-----------|
| Manganese | 10 to 22  |
| 40 Nickel | 1 to 10   |
| Silicon   | .01 to .5 |
| Carbon    | .1 to .4  |
| Iron      | remainder |

45 and the low-expansion member having substantially the following composition

|           | Per cent  |
|-----------|-----------|
| Nickel    | 26 to 45  |
| Cobalt    | 2 to 19   |
| Manganese | .2 to .9  |
| 50 Carbon | .1 to .3  |
| Iron      | remainder |

In testimony whereof, I have hereunto subscribed my name this 18th day of April 1930.

55 HOWARD SCOTT.